

## UNITED STATES PATENT OFFICE

WILLIAM F. RICHTER, OF APOLLO, PENNSYLVANIA, ASSIGNOR TO CHEMICAL HOLDING CORPORATION, OF APOLLO, PENNSYLVANIA, A CORPORATION OF DELAWARE

## PROCESS OF TREATING CELLULOSE MATERIAL

No Drawing.

Application filed June 27, 1929. Serial No. 374,275.

This invention relates to the manufacture of artificial silk and more particularly to a process of treating cellulose material, such as wood pulp, in the manufacture of artificial silk whereby the final filaments or threads produced will possess increased wet and dry strength.

The principal object of this invention is to provide a process of treating cellulose material in the manufacture of artificial silk to produce a final product of superior quality, particularly as regards to strength.

An important object of this invention is to provide an improved method of mercerizing cellulose material particularly for use in the manufacture of artificial silk.

Other objects and advantages of this invention will become apparent during the course of the following description.

In most processes heretofore employed for the manufacture of artificial silk fibrous cellulose material is ordinarily subjected in the initial stages of the process to a mercerizing treatment in a hot solution of caustic. This general procedure is standard practice in the manufacture of rayon according to the so-called "viscose process". Various modifications of the general procedure have been suggested and employed for various purposes.

However, I have found that all of the mercerizing methods commonly employed are disadvantageous in varying degrees because of the fact that partial disintegration of the cellulose due to the excessive shortening of the cellulose molecule results from the present practice. This disintegration eventually results in the production of artificial filaments or threads which are insufficiently strong, particularly when in wet condition, to meet all of the needs of the trade.

I have discovered that the disintegration referred to and its resulting disadvantageous results may be materially decreased by a simple modification of the standard practice, and it is the principal purpose of this invention to provide a simple and efficient process of treating cellulose material, such as sulphite pulp, to produce an alkali cellulose which when treated according to standard practice of making artificial silk will produce fila-

ments or threads which are of a superior strength both in the wet and dry condition.

In the preferred practice of my process I first immerse cellulose fiber, particularly wood pulp or wood pulp mixed with clean cotton dust as described and claimed in my copending application Serial No. 374,276, filed June 27, 1929, in an aqueous solution of caustic, such as sodium hydroxide, of suitable strength for a relatively short period of time at substantially normal atmospheric temperature. Thereafter the pulp is pressed to remove the excess of caustic, the actual amount of pressing being such that for each part of cellulose there will remain approximately from one to three parts of caustic, computed as free caustic on a dry basis. The resulting product is then ground either in the usual manner or in the preferred manner hereinafter described for approximately two and one-half hours, after which the alkali cellulose formed is aged for approximately from twenty-four to forty-eight hours at ordinary atmospheric temperature. The alkali cellulose thus prepared is then in condition for the customary chemical treatment to convert the cellulose material into a spinning solution. Since this subsequent treatment forms no part of this invention per se, and since the alkali cellulose prepared may be treated according to standard practice, a specific description of the actual process of converting the alkali cellulose into a spinning solution and forming such solution into artificial silk need not be set forth.

While numerous obvious modifications may be made in the process, the following specific procedure may be considered as illustrative of the invention although it is to be clearly understood that the invention is not to be limited thereto:

The cellulose fiber to be treated, such as sulphite pulp manufactured from spruce or poplar wood, is immersed in an aqueous solution of sodium hydroxide. Such solution containing from about 17 to 19 per cent by weight of sodium hydroxide. In the preferred practice of my invention an 18 per cent. solution of caustic soda is employed. The amount of cellulose material immersed in the

caustic solution is preferably in the proportions of one part of cellulose material to from fifteen to twenty-five, and preferably twenty, parts by weight of the caustic solution. This treatment is conducted at ordinary atmospheric temperature, preferably between 17° and 20° C., for a period of approximately fifteen minutes. The best results are obtained by conducting the treatment for this period of time, although treatment for a greater period of time, not to exceed forty-five minutes, may be employed in some instances according to the material being treated. Obviously treatment for a slightly less period of time than that indicated as the preferred time may be employed although satisfactory results are not obtained if the cellulose material is kept immersed in the caustic solution for too short a period.

The thus treated material is then pressed to remove the excess of caustic soda. As stated above, I prefer to press the material to such an extent that there will remain for each part of cellulose from one to three parts by measure of caustic soda computed as free caustic on a dry basis. The pressed material is then introduced into a conventional grinder where it is ground for a period of approximately two and one-half hours. I have found that in grinding alkali cellulose after removal of the excess caustic it is highly advantageous to periodically reverse the direction of rotation of the grinding element. Thus in accordance with the invention the grinding operation is effected in repeated cycles of alternated grinding direction. Preferably, the grinding element is rotated in opposite directions for relatively short periods of time, for example three minutes in one direction and then five minutes in the other direction, this cyclic alternating grinding being continued throughout the indicated grinding time, which usually is about two and one-half hours.

This repeatedly alternated rotation grinding procedure prevents packing of the alkali cellulose in the drum, by frequently and repeatedly breaking up the compact crumb aggregates which form. In consequence there results a more rapid and uniform interpenetration of and attack by the alkali than has been the case in the prior practice, in which the grinding element is operated continuously in one direction for about two hours, and then in the opposite direction during the last one-half hour. One result of my new repeatedly alternated rotation grinding is that the steeping time may be reduced to the period described above. Also, the greater uniformity which results from such grinding reduces the time of aging. A major advantage of this procedure, in addition to the foregoing economically important benefits, is that it exerts a beneficial effect upon the product, by giving a rayon whose physical properties, in

both the wet and the dry condition, are improved materially over those obtained by the prior grinding procedures. The ground material which consists substantially entirely of alkali cellulose is then aged for from twenty-four to forty-eight hours at ordinary temperature. Thereafter the aged material is treated in any suitable conventional manner to prepare artificial silk therefrom.

The above described process is particularly adapted for use where wood pulp or wood pulp mixed with cotton dust is used as raw material but it is also adapted for use with numerous other cellulose fibers. However, I have found that when cotton linters are treated according to this process no particularly advantageous results are obtained over the usual process and accordingly I do not recommend the use of the process for treating cotton linters.

While I have described in detail the preferred practice of my process, it is to be understood that the details of procedure may be variously modified without departing from the spirit of the invention or the scope of the subjoined claims.

What I claim is:

1. In the preparation of viscose by treating cellulose fiber with caustic soda and grinding the alkali cellulose thus formed, the step comprising reversing the direction of grinding at continuously repeated relatively short intervals of time.

2. In the preparation of viscose, the steps comprising treating wood cellulose fiber with an approximately 18 per cent solution of sodium hydroxide, removing the excess sodium hydroxide, grinding the alkali cellulose thus formed by repeatedly reversing the direction of grinding at relatively short intervals of time until grinding is complete.

3. In the preparation of viscose by treating wood cellulose fiber with caustic soda and grinding the alkali cellulose thus formed, the step comprising repeatedly reversing the direction of grinding at relatively short intervals of time, and continuing such repeated alternation of grinding direction for about two and one-half hours.

4. In the preparation of viscose by treating cellulose fiber with caustic soda and grinding the alkali cellulose thus formed, the steps comprising grinding the alkali cellulose in one direction for about five minutes, then reversing the direction of grinding for about three minutes, and continuously repeating such reversal of grinding direction until grinding is complete.

5. In the preparation of viscose, the steps comprising treating cellulose fiber with an approximately 18 per cent solution of sodium hydroxide at atmospheric temperature during about 15 to 45 minutes, removing the excess sodium hydroxide and grinding the alkali cellulose by repeatedly reversing the direction

of grinding at relatively short intervals of time.

6. In the preparation of viscose, the steps comprising treating cellulose fiber with an approximately 18 per cent solution of sodium hydroxide at atmospheric temperature during about 15 to 45 minutes, removing the excess sodium hydroxide, and grinding the alkali cellulose in one direction for about 5 minutes, then reversing the direction of grinding for about three minutes, and repeating such reversal of grinding direction for about two and one-half hours.

7. A process of preparing alkali cellulose for use in viscose manufacture, comprising treating a mixture of wood cellulose fiber and cotton dust the fibers of which are shorter than said wood fiber with an approximately 18% solution of sodium hydroxide, removing the excess sodium hydroxide, and grinding the thus-treated cellulose and during such grinding repeatedly reversing the direction of grinding at relatively short intervals of time.

In testimony whereof I affix my signature.

25 WILLIAM F. RICHTER.

30

35

40

45

50

55

60

65